

## 1

2,803,171

PROCESS FOR PRODUCING A WATER VAPOR  
IMPERMEABLE BOARD

Richard H. Cubberley, Morris Township, and M. Benjamin Dell, Morristown, N. J., assignors to The Patent and Licensing Corporation, New York, N. Y., a corporation of Massachusetts

No Drawing. Application August 26, 1953,  
Serial No. 376,749

1 Claim. (Cl. 92—41)

The present invention relates to an improved paper or paper board which is water vapor impermeable, and to a process for producing it.

Water vapor impermeable multi-ply paper or paper board such as box board, is manufactured by forming a plurality of plies on a cylinder type paper making machine and applying a film of emulsified bitumen between selected plies of the sheet simultaneously with the formation thereof. The water proofing film is commonly applied as a bituminous layer interposed between two of the cylinder moulds of the paper making machine. Emulsion applicator units which are used for this purpose comprise essentially a screen-covered roll which continuously revolves in a body of bituminous emulsion, maintained in a suitable trough. A film of the emulsified bitumen is picked up by the screen on the roll and is transferred to the surface of a wet fibrous ply as it passes over the applicator roll. Fresh supplies of the emulsion of the requisite consistency are passed into the trough as the emulsion is taken up by the roll.

Process and apparatus for coating the wet plies in this manner are described, for example, in U. S. Patents Nos. 1,686,818; 1,722,432; 1,724,137 and 1,732,361 and more recent improvements are found in U. S. Patents Nos. 2,622,313 and 2,622,491. This has provided a material which is resistant to the passage of water vapor and wherein the vapor-proofing medium is inexpensively applied and substantially protected from removal when the board is folded, as might be the case with surface coated board. The bituminous material is of such a nature that the coating between the plies does not initially prohibit the water from draining off the paper, and yet after passing through drier rolls, a continuous film is formed which is resistant to the passage of water vapor.

While this process and the product thereof has been found highly successful for many years, nevertheless, in certain applications such as containers for food, it is more desirable to have a material not possessing the black color of the bitumen and having a somewhat greater water vapor impermeability. Furthermore, in many applications it is desirable to have a grease barrier such as in the packaging of doughnuts, potato chips, etc. Such a product should contain all of the other desirable features of the bituminous coating process, including the fact that the coating does not come in contact with the contents of the containers which may be made from the board, and also does not interfere with the printing, folding or gluing of the board.

It is, therefore, a principal object of the present invention to provide an improved paper board which is water vapor impermeable.

It is a further object of the present invention to provide an improved paper board which is resistant to the passage of grease.

It is a further object of the present invention to provide a paper board having a material applied between the plies thereof which is light in color, folds without cracking, and is water vapor impermeable.

## 2

It is a further object of the present invention to provide an improved process for making paper board, including the application to the wet plies thereof, of a material which forms a film in the dry board which is of a light color, resistant to the passage of grease, folds without cracking, and is impermeable to water vapor.

These and other objects are attained by the present invention which relates to an improved paper board within which is a film of a composition comprising a major proportion of wax, a minor proportion of solid homopolymer of isobutene, copolymer of isobutene with approximately 2.5% of isoprene or polyethylene and mixtures thereof and clay.

The water vapor impermeable film is put on the wet plies of the board in the form of an emulsion, utilizing clay as the emulsifying agent, together with a cationic promoter. The clay is desirable in that it forms an emulsion which does not migrate substantially in the paper, and permits the paper to drain before drying.

In order to obtain the desirable ratio of isobutene polymer or polyethylene and wax to clay, it has been found necessary to utilize a cationic promoter. For example, a ratio of 2½ parts of isobutene polymer and wax to 1 part of kaolin clay will form an unstable emulsion without a promoter. However, in order to obtain ratios of 3 to 10 parts of isobutene polymer wax per part of kaolin clay in a stable emulsion, it is necessary to use a promoter. It has been found that a cationic promoter such as an alkyl amine is effective.

Petroleum waxes may be used, including paraffin wax, but microcrystalline wax is preferable, since it gives a film which does not crack or craze easily.

The clay is selected from the group consisting of ball clay and kaolin clay, but kaolin clay has been found preferable. The clay stabilized emulsion on drying forms a film which will not flow under heat because of the honey-comb structure of the film. Clays such as bentonite are not desirable because of the difficulty of drainage due to highly colloidal gels which are formed and which may permit the sheet to separate.

The isobutene polymer should be a substantially solid material which is somewhat elastomeric in nature, having a molecular weight in the range 30,000 to 150,000. The polyethylene should be a substantially solid resinous material, or in other words, having a molecular weight in the range 7,000 to 25,000. The invention is primarily concerned with either of these two materials or with mixtures thereof, or with mixtures of either one and small amounts of other resins. Preferably, however, substantially pure isobutene polymer is used. The most preferable material is GRI or butyl rubber, which is a copolymer of substantially pure isobutene copolymerized with approximately 2.5% of isoprene. Another suitable commercial product is known as "Vistanex," which is similar to the butyl rubber but does not contain isoprene.

The amount of polymer should be in the range 5 to 45% of the total polymer wax composition, and is preferably about 25%. Mixtures of the two polymers found particularly suitable include 5 parts polyethylene, 20 parts isobutene polymer and 75 parts wax. In any case, a desirable composition of polymer and wax should have a viscosity of about 100,000 centipoises at 180 to 220° F.

The cationic promoter may be any cationic surface active agent. Of these, it has been found preferable to use an amine known commercially as "Armeen H. T. D.," which is approximately 25% hexadecyl amine, 70% octadecyl amine and 5% octadecenyl amine. The cationic surface active agents are illustrated by the following:

A. Aliphatic amines and their derivatives.  
Dodecylamine

- B. Homologs of aromatic amines having fatty chains.  
Dodecylaniline
- C. Fatty amides derived from aliphatic diamines.  
Undecylimidazoline
- D. Fatty amides derived from disubstituted diamines.  
Oleylaminodiethylamine
- E. Quaternary ammonium salts and hydrates.  
Triethyl cetyl ammonium iodide
- F. Amides obtained from amino alcohols and their quaternary ammonium derivatives.  
Dimethylstearyl hydroxyethyl ammonium
- G. Quaternary ammonium bases derived from the fatty amides of disubstituted diamines.
- H. Fatty amides derived from benzimidaxolines.



- I. Basic pyridinium compounds and their salts.  
Octadecyl methylene pyridinium acetate
- J. Basic sulfonium, phosphonium and antimonium compounds.  
Methyl sulfate of dimethyloctadecyl sulfonium
- K. Betaine compounds of quaternary ammonium.  
Hydrochloride of dimethyloctadecylmethyl amino-acetate
- L. Dimethylphenylbenzyl ammonium chloride.
- M. Urethanes or basic salts of ethylene diamine.  
Menthol diurethane hydrochloride
- N. Polyethylene diamines and their quaternary ammonium derivatives.
- O. Polypropanol polyethanolamines.

#### EXAMPLE

All equipment should be clean to prevent discoloration of the emulsion. The water used should be substantially free of sulfur compounds.

##### *Preparation of master batch*

|                                                              | Parts |
|--------------------------------------------------------------|-------|
| Polyisobutene (GRI-17)-----                                  | 96.5  |
| Microcrystalline wax M. P.—180° F., 30 pen. at<br>77° F----- | 53.5  |

The polyisobutene was placed in a slightly warm Banbury mixer. The batch was mixed until the temperature rose to 250–300° F. and then about 1/4 of the total wax was added. This was repeated 3 times, the wax being added only when the temperature was between 250 and 300° F.

##### *Preparation of emulsion*

|                                                                                                                                        | Parts |
|----------------------------------------------------------------------------------------------------------------------------------------|-------|
| Master batch-----                                                                                                                      | 150   |
| Microcrystalline wax-----                                                                                                              | 236   |
| Alkyl amine (Armeen H. T. D.)-----                                                                                                     | 0.2   |
| Clay slip at 210° F:<br>77.1 parts of kaolin clay (Crossman clay)<br>154.2 parts water                                                 | 55    |
| Lignin sulphonate: 0.25 part of lignin sulphonate<br>(Marasperse N) was dissolved in 1 part of water<br>heated between 140 and 150° F. | 60    |
| Water -----                                                                                                                            | 223   |

The master batch was mixed with about 45 parts wax in a Baker-Perkins dispersion mixer heated to about 100 to 120° F. When a homogeneous blend was produced, 45 parts more of wax were added. As soon as the blend again became homogeneous, the remainder of the wax was added. After waiting several minutes and then raising the temperature of the blend to 195–200° F., the alkyl amine was added. At this point the mixer was stopped

- and the entire clay slip quickly added. The mixer was immediately started and the temperature maintained at 180° F. after which the blend inverted. After a few minutes the mixture assumed a homogeneous appearance and part of the water at 210° F. was added gradually for several minutes. Thereafter, the rest of the water at room temperature was added and the lignin sulphonate solution added. The emulsion was passed through a 30 mesh screen and stored in polyethylene lined drums.
- 10 The emulsion of this example was diluted with equal parts of water and delivered to an application apparatus on a paper machine of the type adapted to apply bituminous emulsion to wet plies. The usual device for application is a wire covered cylinder immersed in a bath of the emulsion maintained at a constant level. The finished board made on the machine was tested after passing through the drying rolls and stacked in the usual manner. Examination of the sheet showed that the film had not migrated, and the plies adhered satisfactorily.
- 15 20 Water vapor permeability tests were made by covering weighed dishes of anhydrous calcium chloride with samples of board, placing the dishes in a constant humidity apparatus such as the General Foods cabinet, and then weighing the dishes again at stated time intervals. The tests are ASTM tests D988-51T. The average water vapor transmission of the sheet was very low, averaging about 0.4 gram of water per 100 square inches of board per 24 hours at 100° F. with 90% relative humidity for 10 lbs. blend per 1000 square feet of board. This compares with a moisture vapor transmission of 2.5 grams for a coverage of about 20 lbs. per 1000 square feet of bitumen.

We claim:

- 35 A process for producing a water vapor impermeable paper board comprising applying to a wet inner ply of the board on a cylinder machine an emulsion comprising water, a major proportion of petroleum wax, a minor proportion of a solid polymer selected from the group consisting of homopolymers of isobutene, copolymers of isobutene with approximately 2.5% of isoprene and polyethylene and mixtures thereof, a clay selected from the group consisting of kaolin and ball clay, and a cationic surface active agent, and wherein the ratio of the combined wax and polymer is 3 to 10 parts per part of clay, applying at least one ply over the emulsion, draining the water and drying the board in the usual manner.

#### References Cited in the file of this patent

##### UNITED STATES PATENTS

- |            |                       |                |
|------------|-----------------------|----------------|
| Re. 15,461 | Perry -----           | Sept. 26, 1922 |
| 58,944     | Hurlbut -----         | Oct. 16, 1866  |
| 852,918    | White -----           | May 7, 1907    |
| 1,616,902  | Kirschbraun -----     | Feb. 8, 1927   |
| 1,621,888  | Kirschbraun -----     | Mar. 22, 1927  |
| 2,343,090  | Smith -----           | Feb. 29, 1944  |
| 2,343,095  | Smith -----           | Feb. 29, 1944  |
| 2,416,447  | Laughlin et al. ----- | Feb. 25, 1947  |
| 2,487,899  | Sherman -----         | Nov. 15, 1949  |
| 2,492,702  | Neubert et al. -----  | Dec. 27, 1949  |
| 2,493,604  | Walters -----         | Jan. 3, 1950   |
| 2,510,661  | Safford -----         | June 6, 1950   |
| 2,563,897  | Wilson et al. -----   | Aug. 14, 1951  |
| 2,582,037  | Hyde -----            | Jan. 8, 1952   |
| 2,610,939  | Fisher -----          | Sept. 16, 1952 |
| 2,626,213  | Novak -----           | Jan. 20, 1953  |
| 2,649,386  | Snowman -----         | Aug. 18, 1953  |
| 2,658,828  | Pattilloch -----      | Nov. 10, 1953  |

##### FOREIGN PATENTS

- |                     |               |
|---------------------|---------------|
| Great Britain ----- | Apr. 12, 1922 |
| Great Britain ----- | Jan. 2, 1952  |